

## 1

3,149,012  
SMOKELESS POWDER CONTAINING  
ACRYLIC POLYMERS

Ralph F. Preckel, Cumberland, Md., assignor, by mesne assignments, to the United States of America as represented by the Secretary of the Navy  
No Drawing. Filed Nov. 14, 1955, Ser. No. 546,763  
11 Claims. (Cl. 149—98)

This invention relates to the manufacture of smokeless powder and more particularly to an improved "solvent" process for manufacturing smokeless powder and the improved products obtained therefrom.

Currently, smokeless powder is prepared either by the "solvent" process, by "solventless extrusion," or by a casting procedure. In the "solvent" process, nitrocellulose is dissolved in or colloided by the addition thereto of a volatile solvent such as acetone, ether-alcohol, acetone-alcohol, and the like, and by mixing the nitrocellulose and solvent until a viscous or doughy mass is obtained. This mass is then granulated by extrusion and cutting or other suitable means and the volatile solvent is removed as completely as possible. While this process has been a standard means for producing smokeless powder, particularly in small granulations, it has always been recognized that the amount of time necessary to extract the volatile solvent from the grains is undesirably great. It is an accepted fact that the volatile solvent, because of its great affinity for nitrocellulose, is never completely removed from the grains in any practical drying time and that even in small granulations residual solvent migration results in changes in ballistics. Because of the great difficulty in removing the volatile solvent, the process is not used where a powder web of greater than 0.5 inch is desired.

Because of the limitations of the currently known "solvent" process, the "solventless extrusion" techniques were developed. In the conventional "solventless extrusion" method, the desired powder ingredients are mixed in the presence of water. The resulting paste or slurry is then dried to the desired moisture content and the resulting mass is rolled on hot rolls to obtain a colloided sheet. This sheet is then extruded or flaked into the desired granulation. While it has been necessary to employ this process in place of the "solvent" process where a powder web of greater than about 0.5 inch is desired, it has long been recognized that the "solventless extrusion" process leaves much to be desired from the viewpoint of a facile manufacturing operation. For example, in "solventless extrusion" techniques poor quality is occasionally caused in the extruded grains by air which is trapped within the charge prior to extrusion. Moreover, the large amount of manual handling involved makes the "solventless extrusion" process relatively expensive.

When even larger powder grains with even thicker webs became desirable for use in rockets and in JATO units, it was recognized that due to the massive nature of the extrusion presses which would be necessary to produce such large grains, including handling and preforming for the press charge, even the "solventless extrusion" process was unsatisfactory. As a result, several casting techniques have been developed in which small granules, usually

## 2

manufactured by the "solvent" process, are introduced into a mold together with the desired explosive and non-explosive nonvolatile plasticizers and a grain of the desired size is cast by the solvation of the granules by the plasticizer. However, in order to produce a cast grain in this manner, it is necessary to accept the disadvantages of either the "solvent" and "solventless extrusion" processes in the production of the base grain to be used in the casting operation.

Now in accordance with the present invention, a process has been discovered which permits manufacturers of smokeless powder to take advantage of the desirable characteristics of the "solvent" process and yet avoid the presence of volatile constituents in the finished product. Furthermore, the process leads to a new article of manufacture comprising granulated smokeless powder substantially free of volatile constituents.

Generally described, the present invention is a process for manufacturing smokeless powder which comprises forming a uniform doughy mass containing from 15-50% of nitrocellulose, from 15-60% of liquid explosive nitric ester and from 5-30% of at least one catalyzed liquid polymerizable material of the group consisting of the methyl, ethyl, propyl, butyl, and isobutyl esters, and the nitriles of acrylic and methacrylic acids, extruding the mass and cutting into the desired granulation, and curing the grains at a temperature of above 20° C. and below the ignition point of any of the ingredients to form a polymerized product substantially free from volatile constituents. The present invention further contemplates the novel products thus produced.

Having generally described the invention, the following examples are given to illustrate specific embodiments of the invention.

In Table 1, data are given which compare the performance in cal. .30 cartridges of a standard single-base powder with a powder of comparable potential formulated and produced in accordance with the invention. The powders had the following formulations:

|                              | Standard                           | Invention                                              |
|------------------------------|------------------------------------|--------------------------------------------------------|
| 45 Nitrocellulose (13.25% N) | 85.0%                              | 38.0%                                                  |
| Dinitrotoluene               | 10.0%                              |                                                        |
| Diethylphthalate             | 5.0%                               |                                                        |
| Diphenylamine                | 1.0% (Added)                       |                                                        |
| Ethyl Centralite             |                                    | 1.0%                                                   |
| Nitroglycerin                |                                    | 40.0%                                                  |
| 50 Solvent                   | 70 parts, Ether/<br>Alcohol 65/35. | 21.0% (Polymer-<br>izable—contains<br>0.5-1.0%) (cat.) |

55 In both cases the powder ingredients were mixed in a Werner-Pfleiderer type sigma blade mixer until a uniform dough was obtained. This dough was extruded in a hydraulic press and cut into grains. The green grains of standard powder were air dried for two days, water dried for five days, and then air dried two more days to remove the colloiding solvent. The green grains of the powder of the invention were cured in a sodium chloride brine maintained at a temperature of 80° C. for 8 hours. The

powders were loaded in cal. .30 components and fired with the following results:

Table 1

| Example  | Solvent     | Cut<br>Grain Dia.,<br>Pin Dia. | Charge<br>Weight<br>(gr.) | Air<br>Space | No.<br>Shots | Mean<br>Velocity,<br>ft./sec. | Mean<br>Pres-<br>sure,<br>p.s.i. | Catalyst,<br>percent |
|----------|-------------|--------------------------------|---------------------------|--------------|--------------|-------------------------------|----------------------------------|----------------------|
| Standard | Ac/alc.     | 16<br>0.053-.015               | 52.0                      | -0.02        | 5            | 2,346                         | 43,700                           | -----                |
| 1        | MMA         | 16<br>0.053-.015               | 48.0                      | -0.03        | 5            | 2,183                         | 44,900                           | (A) 1.0              |
| 2        | MMA         | 16<br>0.040-.010               | 55.0                      | 0.00         | 5            | 2,264                         | 44,100                           | (A) 1.0              |
| 3        | MA          | 32<br>0.040-.010               | 31.0                      | +.74         | 5            | 2,351                         | 41,600                           | (A) 0.5              |
| 4        | EA          | 32<br>0.040-.010               | 32.5                      | +.69         | 5            | 2,354                         | 39,100                           | (A) 0.5              |
| 5        | BA          | 32<br>0.040-.010               | 36.5                      | +.39         | 5            | 2,349                         | 44,500                           | (A) 0.9              |
| 6        | AN/MA-30/70 | 32<br>0.040-.010               | 32.0                      | +.69         | 5            | 2,398                         | 44,100                           | (A) 0.5              |
| 7        | AN/EA-30/70 | 32<br>0.040-.010               | 36.0                      | +.54         | 5            | 2,331                         | 43,300                           | (A) 0.5              |
| 8        | MA/SP-50/50 | 32<br>0.040-.010               | 40.0                      | +.35         | 5            | 2,499                         | 48,200                           | (A) 1.0              |

Ac/alc.—acetone/alcohol.

MMA—methyl methacrylate.

MA—methyl acrylate.

EA—ethyl acrylate.

BA—butyl acrylate.

AN—acrylonitrile.

SP—styrene polyester (styrene/ethylene glycol maleate-30/70).

(A) Luperco ATC (50/50 mixture of benzoyl peroxide and tricresyl phosphate).

In Table 2, data are given which compare the performance in cal. .30 cartridges of a standard double base powder and another series of powders of the invention of comparable potential. The powders had the following formulations:

|                           | Standard                         | Invention                                    |
|---------------------------|----------------------------------|----------------------------------------------|
| Nitrocellulose (13.25% N) | 81.98%                           | 34.00%                                       |
| Nitroglycerin             | 15.0%                            | 50.0%                                        |
| Diphenylamine             | 0.6%                             | 1.0%                                         |
| Ethyl Centralite          | 1.40%                            | 1.0%                                         |
| Barium Nitrate            | 0.75%                            | 15 (Polymerizable—contains 0.5-1.0%) (cat.). |
| Solvent                   | 57 parts, Acetone/Alcohol 50/50. |                                              |

The powders were prepared by the same processes used in producing the powders of Examples 1-8.

In Table 3, data are presented which compare the performance in cal. .30 cartridges of a standard triple base

solventless powder and a powder of the invention of comparable potential. The two powders had the following compositions:

|    | Standard                  | Invention                                                                      |
|----|---------------------------|--------------------------------------------------------------------------------|
| 35 | Nitrocellulose (13.25% N) | 20.0%                                                                          |
|    | Nitroglycerin             | 19.0%                                                                          |
|    | Ethyl Centralite          | 6.0%                                                                           |
|    | Nitroguanidine            | 54.7%                                                                          |
|    | Solvent                   | 15 parts, Acetone/Alcohol 70/30.                                               |
| 40 |                           | 20.0%<br>30.0%<br>1.0%<br>34.0%<br>15.0% (Polymerizable—contains 1.0%) (cat.). |

The standard powder was prepared by the techniques previously described. The powder of the invention was prepared by the process used in producing the powders of Examples 1-19.

Table 2

| Example  | Solvent     | Cut<br>Grain Dia.,<br>Pin Dia. | Charge<br>Weight<br>(gr.) | Air<br>Space | No.<br>Shots | Mean<br>Velocity,<br>ft./sec. | Mean<br>Pres-<br>sure,<br>p.s.i. | Catalyst,<br>percent |
|----------|-------------|--------------------------------|---------------------------|--------------|--------------|-------------------------------|----------------------------------|----------------------|
| Standard | Ac/alc.     | 16<br>0.053-.015               | 39.0                      | +.46         | 5            | 2,585                         | 53,900                           | -----                |
| 9        | EMA         | 16<br>0.040-.010               | 45.0                      | +.14         | 3            | 2,161                         | 45,500                           | (A) 1.0              |
| 10       | MMA         | 16<br>0.040-.010               | 51.0                      | +.13         | 5            | 2,716                         | 52,800                           | (A) 1.0              |
| 11       | EMA         | 16<br>0.040-.010               | 49.0                      | +.11         | 5            | 2,635                         | 51,800                           | (A) 1.0              |
| 12       | MA          | 16<br>0.040-.010               | 36.5                      | +.51         | 5            | 2,660                         | 52,500                           | (A) 0.5              |
| 13       | EA          | 16<br>0.040-.010               | 37.0                      | +.51         | 5            | 2,626                         | 48,800                           | (A) 0.5              |
| 14       | AN/MA-35/70 | 16<br>0.040-.010               | 39.0                      | +.36         | 5            | 2,679                         | 55,900                           | (A) 0.5              |
| 15       | AN/EA-30/70 | 16<br>0.040-.010               | 41.5                      | +.30         | 5            | 2,685                         | 55,900                           | (A) 0.5              |
| 16       | MMA         | 16<br>0.040-.010               | 50.0                      | +.03         | 5            | 2,563                         | 51,800                           | (A) 1.0              |
| 17       | EMA         | 16<br>0.040-.010               | 48.5                      | +.02         | 5            | 2,580                         | 52,300                           | (A) 1.0              |
| 18       | MA/SP-50/50 | 16<br>0.040-.010               | 45.0                      | +.14         | 6            | 2,805                         | 57,200                           | (A) 1.0              |
| 19       | EMA         | 16<br>0.040-.010               | 49.0                      | -.10         | 5            | 2,616                         | 53,300                           | (B) 1.0              |

Ac/alc.—acetone/alcohol.

EMA—ethyl methacrylate.

MMA—methyl methacrylate.

MA—methyl acrylate.

EA—ethyl acrylate.

AN—acrylonitrile.

SP—styrene polyester (styrene/ethylene glycol maleate-30/70).

(A) Luperco ATC (50/50 mixture of benzoyl peroxide and tricresyl phosphate).

(B) Azo-bis-isobutyronitrile.

Table 3

| Example  | Solvent     | Cut<br>Grain Dia.,<br>Pin Dia. | Charge<br>Weight<br>(gr.) | Air<br>Space | No.<br>Shots | Mean<br>Veloci-<br>ty,<br>ft./sec. | Mean<br>Pres-<br>sure,<br>p.s.i. | Catalyst,<br>percent |
|----------|-------------|--------------------------------|---------------------------|--------------|--------------|------------------------------------|----------------------------------|----------------------|
| Standard |             | 16<br>0.053-0.015              | 56                        | .00          | 5            | 2,184                              | 42,800                           | -----                |
| 20       | MMA         | 16<br>0.053-0.015              | 40                        | .00          | 1            | 1,888                              | 34,400                           | (A) 1.0              |
| 21       | MA/SP-30/70 | 32<br>0.040-0.010              | 30                        | .46          | 5            | 2,061                              | 40,600                           | (A) 1.0              |

MMA—methyl methacrylate.

MA—methyl acrylate.

SP—styrene polyester (styrene/ethylene glycol maleate—30/70).

(A) Luperco ATC (50/50 mixture of benzoyl peroxide and tricresyl phosphate).

Table 4

| Formulas                                       | Stand-<br>ard | Ex-<br>ample<br>22 | Ex-<br>ample<br>23 | Ex-<br>ample<br>24 | Ex-<br>ample<br>25 |
|------------------------------------------------|---------------|--------------------|--------------------|--------------------|--------------------|
| Nitroglycerin, percent                         |               | 40.0               | 40.0               | 40.0               | 40.0               |
| Nitrocellulose (13.25% N), percent             | 85.0          | 38.0               | 38.0               | 38.0               | 38.0               |
| Diphenylamine, percent                         | 1.0           |                    |                    |                    |                    |
| Ethyl centralite, percent                      |               | 1.0                | 1.0                | 1.0                | 1.0                |
| Dibutyl phthalate, percent                     |               |                    |                    |                    |                    |
| Dinitrotoluene, percent                        | 5.0           |                    |                    |                    |                    |
| Ethyl methacrylate, percent                    | 10.0          |                    |                    |                    |                    |
| Ethyl acrylate, percent                        |               | 21.0               | 21.0               | 15.0               | 11.0               |
| Acrylonitrile, percent                         |               |                    |                    | 6.0                |                    |
| Styrene/ethylene glycol maleate—30/70, percent |               |                    |                    |                    | 10.0               |
| Die size, 7 perf.                              | .680          | .556               | .556               | .556               | .556               |
| Pin                                            | .072          | .065               | .065               | .065               | .065               |
| Pin circle                                     | .368          | .319               | .319               | .319               | .319               |
| Mixing time, hours                             |               | 4                  | 2                  | 2                  | 2                  |
| Pressing pressure, pounds                      | 1,500         | 500                | 400                | 200                | 600                |
| Curing time, hours                             |               | 8                  | 8                  | 8                  | 8                  |
| Drying time, hours                             | 240           |                    |                    |                    |                    |
| German Test, Mins.                             | 55            | 90+                | 90+                | 90+                | 90+                |
| Determ. Heat of Explosion                      | 720           | 744                | 807                | 914                | 978                |
| Measurements:                                  |               |                    |                    |                    |                    |
| L (Grain length)                               |               | 1.326              | 1.305              | 1.311              | 1.312              |
| D (Grain diameter)                             |               | .5269              | .5252              | .5052              | .5083              |
| d (Perforation diameter)                       |               | .0566              | .0673              | .0640              | .0623              |
| Wo (Outer web)                                 |               | .0934              | .0822              | .0777              | .0654              |
| Wi (Inner web)                                 |               | .0878              | .0953              | .0889              | .0818              |
| Wa (Average web)                               |               | .0906              | .0888              | .0833              | .0816              |
| Closed Bomb Tests:                             |               |                    |                    |                    |                    |
| Relative Quickness                             | 100.0         | 73.58              | 91.36              | 129.39             | 167.26             |
| Relative Force                                 | 100.0         | 103.47             | 109.13             | 122.47             | 118.13             |

Table 5

| Formulas                                       | Stand-<br>ard | Ex-<br>ample<br>26 | Ex-<br>ample<br>27 | Ex-<br>ample<br>28 | Ex-<br>ample<br>29 |
|------------------------------------------------|---------------|--------------------|--------------------|--------------------|--------------------|
| Nitroglycerin, percent                         | 15.0          | 50.0               | 50.0               | 50.0               | 50.0               |
| Nitrocellulose, percent                        | 81.95         | 34.0               | 34.0               | 34.0               | 34.0               |
| Diphenylamine, percent                         | 0.6           |                    |                    |                    |                    |
| Ethyl centralite, percent                      |               | 1.0                | 1.0                | 1.0                | 1.0                |
| Potassium nitrate, percent                     | 0.75          |                    |                    |                    |                    |
| Barium nitrate, percent                        | 1.40          |                    |                    |                    |                    |
| Graphite, percent                              | 0.3           |                    |                    |                    |                    |
| Ethyl methacrylate, percent                    |               | 15.0               |                    |                    |                    |
| Ethyl acrylate, percent                        |               |                    | 15.0               | 10.5               | 7.5                |
| Acrylonitrile, percent                         |               |                    |                    | 4.5                |                    |
| Styrene/ethylene glycol maleate—30/70, percent |               |                    |                    |                    | 7.5                |
| Die size, 7 perf.                              | .680          | .556               | .556               | .556               | .556               |
| Pin                                            | .072          | .065               | .065               | .065               | .065               |
| Pin circle                                     | .368          | .319               | .319               | .319               | .319               |
| Mixing time, hours                             |               | 3                  | 2                  | 2                  | 2                  |
| Pressing Pressure, pounds                      | 400           | 500                | 600                | 250                | 700                |
| Curing time, hours                             |               | 8                  | 8                  | 8                  | 8                  |
| Drying time, hours                             | 240           |                    |                    |                    |                    |
| German Test, Mins.                             | 90+           | 90+                | 90+                | 90+                | 90+                |
| Determ. Heat of Explosion                      | 983           | 970                | 1,052              | 1,147              | 1,164              |
| Measurements:                                  |               |                    |                    |                    |                    |
| L (Grain length)                               |               | 1.322              | 1.322              | 1.311              | 1.325              |
| D (Grain diameter)                             |               | .5371              | .5314              | .5120              | .5156              |
| d (Perforation diameter)                       |               | .0612              | .0501              | .0666              | .0610              |
| Wo (Outer web)                                 |               | .0966              | .0902              | .0793              | .0773              |
| Wi (Inner web)                                 |               | .0700              | .0897              | .0865              | .0872              |
| Wa (Average web)                               |               | .0833              | .0894              | .0829              | .0822              |
| Closed Bomb Tests:                             |               |                    |                    |                    |                    |
| Relative Quickness                             | 100.0         | 87.39              | 107.21             | 127.68             | 134.40             |
| Relative Force                                 | 100.0         | 105.01             | 111.42             | 111.42             | 114.21             |

In Tables 4 and 5, standard single and double base powders and powders prepared in accordance with the invention were produced in cannon granulation. These powders were tested in a du Pont type closed bomb instrumented to give a pressure rate trace in accordance with standard military procurement acceptance testing procedures. Compositions and results are set forth in the tables. 20 The powders of Examples 22-29 were prepared by the same process as Examples 1-21. The polymerizable material of Examples 22-29 contained 1.5-2.0% of Luperco ATC as catalyst. 25

From the foregoing examples, it will be seen that the invention comprises the substitution of certain uniquely operable monomeric polymerizable materials for the conventional volatile colloid solvents heretofore employed by the art. The monomers themselves are volatile but, in accordance with the invention, are polymerized to a polymerization product substantially free from volatile constituents. Thus, it is possible in accordance with the invention to employ conventional mixing apparatus such as a sigma blade mixer, and conventional extrusion presses. It is possible also to employ conventional dry house equipment for the curing step of the process. However, since atmospheric oxygen exhibits an inhibiting effect on the polymerization reaction and extends the drying period, it is preferred to cure the green grains in either an inert gas atmosphere or else in an inert liquid. It is especially preferred to employ a curing bath of a brine solution such as aqueous sodium chloride or potassium sulfate solutions. The preferred curing baths may be heated by conventional means such as by the use of jacketed containers or by the submersion of a waterproof electrical heating unit in the bath itself. 45

The length of the curing step in the process of the invention will depend on the particular monomeric material employed, upon the type and amount of polymerization catalyst, and the temperature employed, which preferably is from 20-100° C. but in all cases below the ignition point of any of the ingredients present. Generally, it has been found that curing can be effected in the order of eight hours and that drying to remove curing water from the powder requires on the average about two days. Thus, 50 the complete processing time as compared to the conventional solvent process is considerably reduced.

The powders of the invention will always contain liquid explosive nitric ester to compensate for the cooling effect of the polymerized solvent which remains in the composition. Thus, all of the powders of the invention are of the multiple base type. As illustrated in Examples 20 and 21 in Table 3, nonaromatic crystalline high explosives, such as nitroguanidine, cyclotrimethylenetriamine, pentaerythritol tetranitrate, ammonium nitrate, and the like, 55 may be included in the composition if desired. Oxygen-carrying salts such as barium nitrate, potassium nitrate, and the like may also be included. These crystalline explosives are incorporated in particulate form in an amount of from 5% to 40% by weight of the powder composition. 60

Conventional deterents and stabilizers may either be added to the composition or employed as coatings as may be desired and by techniques known to the art. Such deterents and stabilizers include diphenylamine, ethyl centralite, the alkyl phthalates such as dibutyl phthalate and resinous materials such as gasoline-insoluble pine wood resin (Vinsol).

Nitrocellulose of any desired degree of nitration may be employed. Generally, however, the nitrogen content will be greater than 11.5% with smokeless nitrocellulose, that is, nitrocellulose having a nitrogen content greater than 12.2% preferred. Nitroglycerin, because of its high potential, is the preferred liquid explosive nitric ester. However, other liquid explosive nitric esters such as ethylene glycol dinitrate, 1,2,3-butanetriol trinitrate, 1,2,4-butanetriol trinitrate, 2-(hydroxymethyl)-2-methyl-1,3-propanediol trinitrate, pentaerythritol trinitrate, dinitroglycerin, and the like may be employed if desired.

As previously indicated, the polymerizable solvent will be selected from the lower alkyl esters and the nitriles of acrylic and methacrylic acids. Other polymerizable materials either do not exert the necessary solvent action on nitrocellulose or else do not polymerize completely at the low temperatures which are necessary in the presence of such explosive materials as nitroglycerin, nitrocellulose and crystalline explosive. Methyl methacrylate and ethyl methacrylate are the preferred monomeric solvents. Mixtures of any of the operable monomers may also be employed. The operable monomers may also be partially polymerized prior to admixture with the remaining ingredients of the powder composition although care must be taken that the mixture does not become too viscous and that the solvent action of the materials is not inordinately affected. Styrene by itself is a poor solvent for nitrocellulose and therefore is not operable per se. Styrene polyesters, although they exhibit excellent curing characteristics at low temperatures, are also inoperable by themselves. However, as illustrated by the examples, excellent compositions can be obtained when styrene polyesters such as styrene/ethylene glycol maleate are employed in admixture with one or more of the operable acrylic esters or nitriles such as acrylonitrile or methacrylonitrile.

Any of the known polymerization catalysts for vinyl type materials may be employed to catalyze the polymerizable material. Such catalysts include benzoyl peroxide, tricresyl phosphate, lauroyl peroxide, methyl ethyl ketone peroxide, tertiary butyl hydroperoxide, di-tert-butyl diterphthalate, and tert-butyl perbenzoate and mixtures thereof. Preferably, the catalysts will be employed in amounts ranging between 0.5% and 2.5% based on the content and type of monomer.

Furthermore, it will be appreciated that in formulation of the powders herein given, there is some loss of monomer solvent by the time the powders are completely processed. This, of course, can be compensated for by adding additional monomer at the time of mixing.

In accordance with the invention herein described and illustrated, the desired solvent process may be employed in the manufacture of smokeless powder without the usual ballistic abberations resulting from the presence of residual volatile solvent. Thus, large grains of smokeless powder for use in rockets and JATO's may be prepared by extrusion of smokeless powder compositions plasticized with polymerizable solvent in accordance with the invention and a casting process need not be employed for grains having large web. Where the smokeless powder in accordance with the invention is employed as base grain in casting techniques, the problem of solvent migration is likewise removed.

Additionally, large web powders and stick powders that are normally made by the solventless process, because of excessive drying time when using the conventional solvent process, can now be made in accordance with this invention by using conventional solvent type equipment and techniques associated with such equipment.

Since modifications of the invention will be apparent to those skilled in the art, it is intended that the scope of the invention be limited only by the appended claims.

10. What I claim and desire to protect by Letters Patent is:
1. A process for manufacturing smokeless powder which comprises forming a uniform doughy mass consisting essentially of from 15 to 50% of nitrocellulose, from 15 to 60% of liquid explosive nitric ester and from 5 to 30% of at least one catalyzed liquid polymerizable material selected from the group consisting of the nitriles of acrylic and methacrylic acids and a styrene polyester and mixtures thereof with lower alkyl acrylates and methacrylates, extruding the mass and cutting into the desired granulation, and curing the grains at a temperature of from about 20° C.-100° C. and below the ignition point of any of the ingredients to form a polymerization product substantially free from volatile constituents.
  2. A process according to claim 1 in which the liquid explosive nitric ester is nitroglycerin.
  3. A process according to claim 1 in which the grains are cured in an inert liquid bath.
  4. A process for manufacturing smokeless powder which comprises forming a uniform doughy mass containing from 15 to 50% of nitrocellulose, from 15 to 60% of liquid explosive nitric ester, from 5 to 40% of particulate crystalline high explosive, and from 5 to 30% of at least one catalyzed liquid polymerizable material of the group consisting of the methyl, ethyl, propyl, butyl and isobutyl esters and the nitriles of acrylic and methacrylic acids, extruding the mass and cutting into the desired granulation, and curing the grains at a temperature of above 20° C. and below the ignition point of any of the ingredients to form a polymerization product substantially free from volatile constituents.
  5. A process according to claim 4 in which the liquid explosive nitric ester is nitroglycerin.
  6. A process according to claim 4 in which the polymerizable material is methyl methacrylate.
  7. A process according to claim 4 in which the polymerizable material is ethyl methacrylate.
  8. A process according to claim 4 in which the grains are cured at a temperature of from 20-100° C.
  9. A process according to claim 4 in which the grains are cured in an inert liquid bath.
  10. As a new article of manufacture, a granulated smokeless powder substantially free of volatile constituents consisting essentially of from 15 to 50% nitrocellulose, from 15 to 60% liquid explosive nitric ester, and from 5 to 30% of at least one polymerized material selected from the group consisting of the nitriles of acrylic and methacrylic acids and a styrene polyester and mixtures thereof with lower alkyl acrylates and methacrylates.
  11. As a new article of manufacture, a granulated smokeless powder substantially free of volatile constituents and comprising from 15 to 50% nitrocellulose, from 15 to 60% liquid explosive nitric ester, from 5 to 40% particulate crystalline high explosive, and from 5 to 30% of at least one polymerized material of the group consisting of the methyl, ethyl, propyl, butyl and isobutyl esters and the nitriles of acrylic and methacrylic acids.

No references cited.